



US00528579A

**United States Patent [19]**

Tanaka et al.

[11] Patent Number: 5,288,579

[45] Date of Patent: Feb. 22, 1994

[54] **DEVELOPER FOR DEVELOPING ELECTROSTATIC IMAGE, IMAGE FORMING APPARATUS, APPARATUS UNIT AND FACSIMILE APPARATUS**

[75] Inventors: **Katsuhiko Tanaka; Kazuyoshi Hagiwara; Tsuyoshi Takiguchi, all of Yokohama; Rika Doi, Tokyo, all of Japan**

[73] Assignee: **Canon Kabushiki Kaisha, Tokyo, Japan**

[21] Appl. No.: **801,486**

[22] Filed: **Dec. 2, 1991**

[30] **Foreign Application Priority Data**

Nov. 30, 1990 [JP] Japan ..... 2-33095  
May 20, 1991 [JP] Japan ..... 3-142763

[51] Int. Cl.<sup>5</sup> ..... **G03G 9/00; G03G 9/083; G03G 9/107**

[52] U.S. Cl. ..... **430/110; 430/106;**

**430/106.6**

[58] Field of Search ..... **430/106, 106.6, 109, 430/110, 137**

[56] **References Cited**

**U.S. PATENT DOCUMENTS**

2,297,691 10/1942 Carlson ..... 95/5  
4,636,451 1/1987 Matkin et al. ..... 430/109  
4,663,263 5/1987 Ikeda et al. ..... 430/110

**FOREIGN PATENT DOCUMENTS**

42-23910 11/1967 Japan .

43-24748 10/1968 Japan .

**OTHER PUBLICATIONS**

Patent Abstract of Japan, vol. 10, No. 290 (P-503) [2346], Oct. 2, 1986 for JPA 61-110157, published May 28, 1986.

Patent Abstracts of Japan, vol. 12, No. 203, (P-715) [3050], Jun. 11, 1988 for JPA 63-5357, published Jan. 11, 1988.

Primary Examiner—Marion E. McCamish

Assistant Examiner—Stephen C. Crossan

Attorney, Agent, or Firm—Fitzpatrick, Cella, Harper & Scinto

[57] **ABSTRACT**

A developer for developing electrostatic images is constituted by toner containing a binder resin and a charge controller. The charge controller comprises an arylurea compound which is an arylurea having at least one electron-attracting group or electron-donating group, or a polyarylurea including such an arylurea as a recurring unit. The arylurea compound is substantially colorless and can have stable but different levels of triboelectric chargeability depending on the substituents.

77 Claims, 7 Drawing Sheets







FIG. 2



FIG. 3



FIG. 4



FIG. 5



FIG. 6



FIG. 7



FIG. 8

**DEVELOPER FOR DEVELOPING  
ELECTROSTATIC IMAGE, IMAGE FORMING  
APPARATUS, APPARATUS UNIT AND  
FACSIMILE APPARATUS**

**FIELD OF THE INVENTION AND RELATED  
ARTS**

The present invention relates to a developer for visualizing electrostatic images in image forming methods, such as electrophotography, electrostatic recording and electrostatic printing, and an image forming apparatus, an apparatus unit and a facsimile apparatus using the developer.

Hitherto, a large number of electrophotographic processes have been described, e.g., in U.S. Pat. No. 2,297,691, Japanese Patent Publication (JP-B) 42-23910 and JP-B 43-24748.

Developing methods used in such electrophotographic processes may be roughly classified into the dry developing method and the wet developing method. The former is further classified into the method using a two-component type developer and a mono-component type developer.

The developer used in the dry developing method comprises a toner which has conventionally comprised fine powder in which a dye or pigment is dispersed in a natural or synthetic resin. For example, a colorant is dispersed in a binder resin such as polystyrene, and particles obtained by micropulverizing the resultant dispersion into sizes of about 1-30 microns are used as the toner. A magnetic toner has been prepared by dispersing magnetic particles in a binder resin. In case of the system employing the two-component type developer, a toner is used generally in mixture with carrier particles, such as glass beads or iron powder.

In any case, the toner is required to have a positive or negative charge depending on the polarity of an electrostatic latent image to be developed.

In order to provide a toner with a charge, it is possible to utilize the triboelectric chargeability of a resin constituting the toner. This method however generally provides only a low charge so that the resultant image after development is liable to be accompanied with fog and unclear. It has been practiced to add a dye or pigment having a chargeability-imparting ability or a charge controller.

The charge controllers known in the art at present may include: metal complex salts of monoazo dyes, metal complex salts of salicylic acid, naphthoic acid and dicarboxylic acids, and copper phthalocyanine pigment.

Among these charge controllers, some are liable to soil a toner-carrying member such as a sleeve or a carrier and therefore a toner using such a charge controller causes a lowering in triboelectric charge leading to an image density decrease as the number of copied sheets is increased. Further, some charge controllers provide only an insufficient triboelectric chargeability which is liable to be affected by changes in temperature and humidity, thus resulting in lower image density according to environmental changes. Some charge controllers have a poor storage stability and cause a lowering in triboelectric chargeability during a long term of storage. Some charge controllers have a poor dispersibility in a resin, so that a toner using the controller is liable to be accompanied with nonuniform triboelectric charges among particles and with fog. Some charge controllers have poor thermal stability and can decompose or

denature, and a toner prepared by re-use of a toner using such a controller is liable to produce reversely charged particles resulting in fog. Some charge controllers are colored and therefore cannot be used in a color toner.

For the above reasons, it is still desired to develop a charge controller having further improved properties.

**SUMMARY OF THE INVENTION**

A generic object of the present invention is to provide a developer for developing electrostatic images having solved the above-mentioned problems.

A more specific object of the present invention is to provide a developer which does not easily soil a developer-carrying member, such as a sleeve or a carrier and does not cause a lowering in triboelectric charge on copying of an increased number of sheets, thus providing a stable image density.

Another object of the present invention is to provide a developer excellent in triboelectric chargeability which is little affected by changes in temperature and humidity.

An object of the present invention is to provide a developer having a good storage stability and a triboelectric chargeability which is free from or accompanied with only little change during long term storage.

An object of the present invention is to provide a developer wherein toner particles containing a charge controller uniformly dispersed within a resin are provided with a uniform triboelectric charge to provide the developer with little tendency of providing fogged images.

An object of the present invention is to provide a developer which contains a charge controller having a good thermal stability and free from decomposition or denaturation during a hot kneading step for toner production, can be recycled and is hardly susceptible to fogging.

An object of the present invention is to provide a developer comprising a color toner containing a colorless or light-colored charge controller.

A further object of the present invention is to provide an image forming apparatus, an apparatus unit and a facsimile apparatus using such a developer as described above.

According to the present invention, there is provided a developer for developing electrostatic images, comprising: a toner containing a binder resin and a charge controller, said charge controller comprising an arylurea compound which comprises an arylurea having at least one electron-attracting group or electron-donating group, or a polyarylurea including such an arylurea as a recurring unit.

According to another aspect of the present invention, there is provided an image forming apparatus, comprising:

an image-bearing for bearing an electrostatic latent image;

charging means for charging the image-bearing member,

latent image-forming means for forming a latent image on the charged image bearing member,

developing means for developing the electrostatic latent image to form a toner image on the image-bearing member,

transfer means for transferring the toner image from the image-bearing member to a transfer-receiving material.

cleaning means for removing a portion of the toner remaining on the image-bearing member.

fixing means for fixing the transferred toner image on the transfer-receiving material under action of heat and pressure;

wherein said developing means retains a developer comprising a toner containing a binder resin and a charge controller, said charge controller comprising an arylurea compound which comprises an arylurea having at least one electron-attracting group or electron-donating group, or a polyarylurea including such an arylurea as a recurring unit.

According to another aspect of the present invention, there is provided an apparatus unit which is to be incorporated so as to form the image forming apparatus described above and comprises the developing means supported integrally together with at least one of the image-bearing member, charging means and cleaning means, so that the apparatus can be arbitrarily connected to or released from an apparatus body including at least the latent image forming means, the transfer means and the fixing means.

According a still further aspect of the present invention, there is provided a facsimile apparatus comprising the above-mentioned image forming apparatus as a printer, and receiving means for receiving image data from a remote terminal.

These and other objects, features and advantages of the present invention will become more apparent upon a consideration of the following description of the preferred embodiments of the present invention taken in conjunction with the accompanying drawings.

#### BRIEF DESCRIPTION OF THE DRAWINGS

FIG. 1 is an FTIR chart of an urea derivative of compound Example 1.

FIG. 2 is an  $^1\text{H-NMR}$  chart of an urea derivative of 40 Compound Example 1.

FIG. 3 is an FTIR chart of an urea derivative of Compound Example 21.

FIG. 4 is an  $^1\text{H}$ -NMR chart of an urea derivative of Compound Example 21.

FIG. 6 is an illustration of an embodiment of the image forming apparatus according to the present invention. 50

FIG. 7 is a partially enlarged view of the developing zone of the apparatus shown in FIG. 6.

FIG. 8 is a block diagram of a facsimile apparatus incorporating such an image forming apparatus as a 55 printer.

## DETAILED DESCRIPTION OF THE INVENTION

As a result of our study, it has been discovered that an 60 arylurea compound comprising an arylurea having at least one electron-attracting group or electron-donating group or a polyarylurea including such an arylurea as a recurring unit is substantially colorless and, when contained in a toner, provides the toner with a sufficient 65 triboelectric chargeability, thus providing a solution to the above-mentioned problems. The present invention is based on the discovery.

It has not been known to use a urea derivative as a charge controller, but an analogous compound, thiourea derivative, has been proposed as a charge controller (Japanese Laid-Open Patent Application (JP-A 61-110157). We have examined the triboelectric chargeability of such thiourea derivatives and found that the thiourea derivatives show a negative triboelectric chargeability which however is insufficient. Further, thiourea derivatives show triboelectric chargeabilities which vary little depending on substitutions introduced thereto, and thus it is difficult to obtain a toner having a desired level of triboelectric chargeability.

As a result of our further study for charge controllers having a sufficient triboelectric chargeability and capable of changing triboelectric chargeabilities varying depending on substituents introduced thereto, we have found a class of urea derivatives. Most urea derivatives are colorless or only lightly colored, even if colored, thus being inclusively regarded as substantially colorless, so that they are optimum as charge controllers for color toners. Urea derivatives are thermally and mechanically stable and do not decompose when stirred in a developing apparatus. Therefore, a color toner obtained by using a urea derivative can always provide clear images regardless of an increased number of copying cycles. Thus, the present invention has been accomplished based on a discovery that a toner containing a class of the urea derivatives according to the present invention is provided with better properties than a toner containing a conventional charge controller.

The arylurea compound used as the charge controller according to the present invention comprises an arylurea having at least one electron-attracting group or electron-donating group or a polyarylurea including such an arylurea as a recurring unit.

The arylurea compound according to the present invention may preferably be an N,N'-bisarylurea derivative represented by the following formula (I) in view of facility of synthesis:



wherein  $Y^1$  and  $Y^2$  denote a phenyl or naphthyl group;  $R^1$  and  $R^2$  independently denote a halogen atom, nitro group, sulfonic acid group, carboxyl group, carboxylic acid ester group, cyano group or carbonyl group;  $R^3$  and  $R^4$  denote a hydrogen atom, alkyl group, alkoxy group, phenyl group capable of having a substituent, or aralkyl group capable of having a substituent;  $R^5$  and  $R^6$  denote a hydrogen atom or  $C_1-C_8$  hydrocarbon group;  $k$  and  $l$  are 0, 1 or 2 satisfying  $k+1 \geq l$ ; and  $m$  and  $n$  are 1 or 2. Examples of the substituent attachable to the phenyl group and aralkyl group may include: halogen atom, nitro group, sulfonic acid group, carboxyl group, carboxylic acid group, cyano group and carbonyl group; of which halogen atom, carboxyl group and carboxylic acid ester group are particularly preferred.

Hereinbelow, some representative examples of the arylurea compound having at least one electron-attracting group preferred in view of, e.g., facility of handling are enumerated hereinbelow, but they are not exhaustive:

Compound Example

(1)



(2)



(3)



(4)



(5)



(6)



(7)



(8)



(9)



(10)



(11)



(12)



(13)



(14)



(15)



-continued  
Compound Example



(17)



(18)



(19)



(20)

Another class of the arylurea compound according to the present invention preferred in view of facility of handling may include an  $N,N'$ -bisarylurea derivative 30 represented by the following formula (II):



wherein Y<sup>1</sup> and Y<sup>2</sup> denote a phenyl group, naphthyl group or anthryl group; R<sup>1</sup> and R<sup>2</sup> independently denote an alkyl group, alkoxy group or amino group; R<sup>3</sup> and R<sup>4</sup> denote a hydrogen atom, alkyl group, alkoxy group, amino group, phenyl group capable of having a substituent, or aralkyl group capable of having a substituent; R<sup>5</sup> and R<sup>6</sup> are a hydrogen atom or C<sub>1</sub>-C<sub>8</sub> hydrocarbon group; k and 1 are 0, 1 or 2 satisfying k+1 $\geq$ 1; and m and n are 1 or 2. Examples of the substituent attachable to the phenyl group or aralkyl group may include: alkyl group, alkoxy group and amino group, of which alkyl group is particularly preferred.

Hereinbelow, some representative examples of the arylurea compound having at least one electron-donative group preferred in view of, e.g., facility of handling are enumerated hereinbelow, but they are not exhaustive:



(21)



(27)



(22) 65



(28)

-continued  
Compound Example

The urea derivative according to the present invention may be synthesized according to an ordinary method, e.g., by reacting an aniline derivative and an isocyanate derivative in benzene as solvent. As a specific example, a parachloro-substituted form of Compound Example (1) was synthesized in the following manner.

372.7 g of 4-chloroaniline and 2.5 liter of benzene were charged in a 4-necked flask, and a solution of 448.7 g of 4-chlorophenyl isocyanate was added dropwise thereto in 40 minutes. At the time of the dropwise addition, heat was evolved to raise the temperature up to 55° C. After the addition, the system was heated under a reflux condition (81° C.) for 1.5 hours of reaction. After cooling, the product was recovered by filtration, washed with methanol until the filtrate became clear, and dried for 42 hours by a hot-air drier at 50° C. to obtain 805 g of grayish white powder.

The product was identified by FTIR (Fourier transform infrared spectroscopy) using an infrared spectrophotometer ("Model 270-30", available from Hitachi Seisakusho K.K.) and <sup>1</sup>H-NMR (nuclear magnetic resonance) using a nuclear magnetic resonance apparatus ("Model R-24B", available from Hitachi Seisakusho K.K.) to obtain charts shown in FIGS. 1 and 2, respectively.

A para-methoxy-substituted form of Compound Example (23) was synthesized in the following manner.

320 g of 4-methoxy aniline and 2.5 liter of benzene were charged in a 4-necked flask, and a solution of 395 g of 4-methoxyphenyl isocyanate in 0.5 liter of benzene was added dropwise thereto in 40 minutes. After the addition, the system was heated under a reflux condition (81° C.) for 1.5 hours. After cooling, the product was recovered by filtration, washed with methanol until the filtrate became clear, and dried for 24 hours by a hot-air drier to obtain 695 g of grayish white powder. The product was identified by FTIR and <sup>1</sup>H-NMR to obtain respective charts shown in FIGS. 3 and 4.

A paramethyl-substituted form a Compound Example (21) was synthesized identified in substantially the same manner as above from 4-methylaniline and 4-methylphenyl isocyanate.

5 The urea derivative according to the present invention may be added to a toner internally or externally. The amount of addition cannot be determined in a unitary way but may depend on several factors of toner production, such as the kind of the binder resin, the presence or absence of optional additives and methods of addition of such additives. In case of internal addition, however, it is preferred to use 0.1-10 wt. parts, more preferably 0.1-5 wt. parts of the urea derivative per 100 wt. parts of the binder resin. In case of external addition, it is preferred to use 0.01-10 wt. parts, more preferably 0.05-1 wt. part, of the urea derivative per 100 wt. parts of the binder resin.

10 In the case of the external addition, it is particularly preferred to attach or embed the urea derivative to the surface of fine toner particles comprising a binder resin and a colorant by using an apparatus as shown in FIG. 5. Referring to FIG. 5, a mixture of a toner and a urea derivative are charged through an inlet 13 and an entrance chamber 9 to a central zone defined by a casing 20 6 of the apparatus, wherein dispersion vanes 3 and blades 4 are rotated about a shaft 1 driven by a motor (not shown) to apply an impacting force to the mixture at an impact zone 8 between the blade 4 and a liner 7. Then, the mixture is withdrawn through an outlet chamber 10, a return pipe 11 and a blower 10 to be recycled to the apparatus. After the treatment, the toner particles carrying the urea derivative are withdrawn from a product withdrawal outlet 10. The blades 4 are supported by a rotor 2 which is placed at a part separated from the outlet chamber 10 by a partition plate 5. During the treatment, the temperature within the apparatus is controlled, as desired, by passing cooling water through a jacket 15.

15 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 991

On the other hand, in order to produce silica fine powder to be used in the present invention through the wet process, for example, decomposition of sodium silicate with an acid represented by the following scheme may be applied:



In addition, there may also be used a process wherein sodium silicate is decomposed with an ammonium salt or an alkali salt, a process wherein an alkaline earth metal silicate is produced from sodium silicate and decomposed with an acid to form silicic acid, a process wherein a sodium silicate solution is treated with an ion-exchange resin to form silicic acid, and a process wherein natural silicic acid or silicate is utilized.

The silica fine powder to be used herein may be anhydrous silicon dioxide (silica), and also a silicate such as aluminum silicate, sodium silicate, potassium silicate, magnesium silicate and zinc silicate.

The silica fine powder may preferably have a specific surface area of at least 30 m<sup>2</sup>/g, more preferably 50-400 m<sup>2</sup>/g, as measured by the BET method according to nitrogen adsorption.

The silica fine powder used in the present invention may have been treated with an agent, such as a silane coupling agent or organic silicon compound, for the purpose of imparting a hydrophobicity, etc. More specifically, silica fine powder may be treated with such a treating agent reactive with or physically adsorbed onto the silica fine powder. Examples of such a treating agent may include: hexamethyldisilazane, trimethylsilane, trimethylchlorosilane, trimethylethoxysilane, dimethyl-dichlorosilane, methyltrichlorosilane, allyldimethyl-chlorosilane, allylphenyldichlorosilane, benzylidimethylchlorosilane, bromomethyldimethylchlorosilane,  $\alpha$ -chloroethyltrichlorosilane,  $\beta$ -chloroethyltrichlorosilane, chloromethyldimethylchlorosilane, triorganosilyl-mercaptans such as trimethylsilylmercaptan, triorganosilyl acrylates, vinylmethylacetoxysilane, dimethylethoxysilane, dimethylidimethoxysilane, diphenyldiethoxysilane, hexamethyldisiloxane, 1,3-divinyltetramethyldisiloxane, 1,3-diphenyltetramethyldisiloxane, and dimethylpolysiloxane having 2 to 12 siloxane units per molecule and containing each one hydroxyl group bonded to Si at the terminal units. These may be used alone or as a mixture of two or more compounds.

The silica fine powder used in the present invention may preferably have a hydrophobicity of 30-80 according to the methanol titration test as measured after such a treatment as described above so as to provide a developer containing the silica fine powder with a sharp and uniform triboelectric chargeability. According to the methanol titration test, the degree of hydrophobicity of the silica fine powder having a hydrophobicity imparted surface is determined.

The methanol titration test used herein may be conducted in the following manner. Sample silica powder (0.2 g) is charged into 50 ml of water in a 250 ml-Erlenmeyer's flask. Methanol is added dropwise from a buret until the whole amount of the silica is wetted therewith. During this operation, the content in the flask is constantly stirred by means of a magnetic stirrer. The end point can be observed when the total amount of the silica powder is suspended in the liquid, and the hydrophobicity is represented by the percentage of the methanol in the liquid mixture of water and methanol on reaching the end point.

The colorant to be used in the developer of the present invention may be one or a mixture of known dyes or pigments including Carbon Black, Lamp Black, Iron Black, ultramarine blue, nigrosine dyes, Aniline Blue, Phthalocyanine Blue, Phthalocyanine Green, Hansa Yellow G, Rhodamine 6G Lake, Chalcooil Blue, Chrome Yellow, Quinacridone, Benzidine Yellow, Rose Bengal, triarylmethane dyes, monoazo dyes and pigments and disazo dyes and pigments.

The binder resin for the developer of the present invention may for example be composed of: homopolymers of styrene and derivatives thereof, such as polystyrene, poly-p-chlorostyrene and polyvinyltoluene; styrene copolymers such as styrene-p-chlorostyrene copolymer, styrene-vinyltoluene copolymer, styrene-vinylnaphthalene copolymer, styrene-acrylate copolymer, styrene-methacrylate copolymer, styrene-methyl- $\alpha$ -chloromethacrylate copolymer, styrene-acrylonitrile copolymer, styrene-vinyl methyl ether copolymer, styrene-vinyl methyl

ketone copolymer, styrene-butadiene copolymer, styrene-isoprene copolymer and styrene-acrylonitrile-indene copolymer; polyvinyl chloride, phenolic resin, natural resin-modified phenolic resin, natural resin-modified maleic acid resin, acrylic resin, methacrylic resin, polyvinyl acetate, silicone resin, polyester resin, polyurethane, polyamide resin, furan resin, epoxy resin, xylene resin, polyvinyl butyral, terpene resin, cumarone-indene resin and petroleum resin.

The binder resin may have been crosslinked, and a crosslinked styrene copolymer is particularly preferred.

Examples of the comonomer constituting such a styrene copolymer together with styrene monomer may include other vinyl monomers inclusive of: monocarboxylic acids having a double bond and derivative thereof, such as acrylic acid, methyl acrylate, ethyl acrylate, butyl acrylate, dodecyl acrylate, octyl acrylate, 2-ethylhexyl acrylate, phenyl acrylate, methacrylic acid, methyl methacrylate, ethyl methacrylate, butyl methacrylate, octyl methacrylate, acrylonitrile, methacrylonitrile, and acrylamide; dicarboxylic acids having a double bond and derivatives thereof, such as maleic acid, butyl maleate, methyl maleate and dimethyl maleate; vinyl esters, such as vinyl chloride, vinyl acetate, and vinyl benzoate; ethylenic olefins, such as ethylene, propylene and butylene; vinyl ketones, such as vinyl methyl ketone and vinyl hexyl ketone; and vinyl ethers, such as vinyl methyl ether, vinyl ethyl ether, and vinyl isobutyl ether. These vinyl monomers may be used alone or in mixture of two or more species in combination with the styrene monomer.

The crosslinking agent may principally be a compound having two or more double bonds susceptible of polymerization, examples of which may include: aromatic divinyl compounds, such as divinylbenzene, and divinylnaphthalene; carboxylic acid esters having two double bonds, such as ethylene glycol diacrylate, ethylene glycol dimethacrylate and 1,3-butanediol dimethacrylate; divinyl compounds, such as divinylaniline, divinyl ether, divinyl sulfide and divinylsulfone; and compounds having three or more vinyl groups. These may be used singly or in mixture.

In the case of using a pressure-fixation system, there may be used a binder resin for a pressure-fixable toner, examples of which may include: polyethylene, polypropylene, polybutylene, polyurethane elastomer, ethylene-ethyl acrylate copolymer, ethylene-vinyl acetate copolymer, ionomer resin, styrene-butadiene copoly-

mer, styrene-isoprene copolymer, linear saturated polyester and paraffins.

The toner constituting the developer according to the present invention can be composed as a magnetic toner by incorporating therein a magnetic material. The magnetic material may be one or a mixture of: iron oxides, such as magnetite,  $\gamma$ -iron oxide, ferrite, and excessive iron-containing ferrite; metals, such as iron, cobalt and nickel, and alloys of these metals with other metals, such as aluminum cobalt, copper, zinc, lead, magnesium, tin, zinc, antimony, beryllium, bismuth, cadmium, calcium, manganese, selenium, titanium, tungsten and vanadium; and mixture of the above. These magnetic materials may preferably have an average particle size of 0.1-1 micron, more preferably 0.1-0.5 micron and may preferably be contained in an amount of 40-150 wt. parts, more preferably 60-120 wt. parts, per 100 wt. parts of the binder resin.

The toner containing the charge controller according to the present invention may have a weight-average particle size of 3-15 microns. In view of the developing performance, it is particularly preferred that the toner has a weight-average particle size of 4-10 microns and contains 12-60% by number of toner particles having a particle size of 5 microns or smaller, 1-33% by number of toner particles having a particle size of 8-12.7 microns, and 2.0 wt. or less of toner particles having a particle size of 16 microns or larger.

While particle size distribution of a toner may suitably be measured by means of a Coulter counter in the present invention, it may be measured in other various manners.

Coulter counter Model TA-II (available from Coulter Electronics Inc.) is used as an instrument for measurement, to which an interface (available from Nikkaki K.K.) for providing a number-basis distribution, and a volume-basis distribution and a personal computer CX-1 (available from Canon K.K.) are connected. For measurement, a 1%-NaCl aqueous solution as an electrolytic solution is prepared by using a reagent-grade sodium chloride. For example, ISOTONR-II (available from Coulter Scientific Japan K.K.) may be used therefor. Into 100 to 150 ml of the electrolytic solution, 0.1 to 5 ml of a surfactant, preferably an alkylbenzenesulfonic acid salt, is added as a dispersant, and 2 to 20 mg of a sample is added thereto. The resultant dispersion of the sample in the electrolytic liquid is subjected to a dispersion treatment for about 1-3 minutes by means of an ultrasonic disperser, and then subjected to measurement of particle size distribution in the range of 2-40 microns by using the above-mentioned Coulter counter Model TA-II with a 100 micron-aperture to obtain a volume-basis distribution and a number-basis distribution.

The developer according to the present invention may also be constituted as a two-component type developer by mixing a toner with a carrier. The carrier particles used for this purpose may be those known in the art including, for example, powder or particles of magnetic metals, such as iron, ferrite and nickel; glass beads; and these particles further coated with resins. Examples of such coating resins may include: styrene-acrylate copolymer, styrene-methacrylate copolymer, other acrylate copolymers and methacrylate copolymers, silicone resin, fluorine-containing resin, polyamide resin, ionomer resin and polyphenylene sulfide resin. These resins may be used singly or in mixture.

The developer according to the present invention may further contain optional additives, examples of

which may include: lubricants, such as zinc stearate; abrasives, such as cerium oxide, and silicon carbide; fluidity-imparting agents, such as aluminum oxide; anti-caking agent; and electroconductivity-imparting agents, such as carbon black and tin oxide. It is also possible to add fine powder of a fluorine-containing polymer, such as polyvinylidene fluoride, as a preferable additive, in order to provide fluidity, abrasive-characteristic and charge-stability.

It is also possible to incorporate a releasing substance in a toner so as to improve the releasability at the time of hot roller fixation. Examples of the releasing substance may include waxy substances, such as low-molecular weight polyethylene, low-molecular weight polypropylene, microcrystalline wax, carnauba wax, sasol wax, and paraffin wax. Such a releasing substance may be added in a proportion of about 0.5-5 wt. % of the toner.

The toner according to the present invention may preferably be prepared through a process wherein the above-mentioned toner constituents are sufficiently blended in a blender such as a ball mill, well kneaded by a hot kneading means such as a hot roller kneader or an extruder, cooled to be solidified, mechanically pulverized and classified to provide a toner. It is however also possible to adopt other methods, such as a method of dispersing constituent materials in a binder resin solution and spray-drying the dispersion; a method of incorporating prescribed materials into a core material, a shell material or both of these constituting a so-called micro-capsule toner; and a polymerization method of dispersing prescribed materials in a monomer constituting the binder resin to form an emulsion or suspension, and polymerizing the emulsion or suspension.

The thus obtained toner may be further blended with other additives as desired by means of a blender, such as a Henschel mixer, to provide a developer according to the present invention.

The developer according to the present invention may be applicable to any known methods of developing electrostatic images inclusive of electrophotography, electrostatic recording and electrostatic printing.

Now, the image forming apparatus according to the present invention will be explained with reference to FIGS. 6 and 7.

The apparatus includes a photosensitive drum 21 of, e.g., an OPC (organic photoconductor) as an electrostatic image-bearing member and a charger 22 for charging the photosensitive drum 21. A prescribed voltage is supplied to the charger 22 from a power supply unit 35. Also a prescribed bias voltage is supplied to a transfer charger 23 as a transfer means from a constant voltage supply 34. Preferred bias conditions include a current value of 0.1-50  $\mu$ A and a voltage value (absolute) of 500 to 4000 volts.

The photosensitive drum 21 surface is charged to, e.g., a negative polarity by the charger 22 connected to the power supply unit 35 (voltage application means) and exposed image light from exposure means 26 as a latent image-forming means to form an electrostatic latent image thereon. Then, the latent image is subjected to, e.g., reverse-development with a monocomponent-type negatively chargeable magnetic developer 30 contained in a developing apparatus 29 equipped with a magnetic iron blade 31 and a non-magnetic developing sleeve 24 (developer-carrying member) containing therein a magnet 240. The developing sleeve 24 comprises, e.g., a cylinder of stainless steel (SUS 304)

having a diameter of 50 mm and plural sphere-traced surface concavities thereon. At the developing station or zone, an alternating bias, a pulsed bias and/or a DC bias is applied between the conductive substrate of the photosensitive drum 21 and the developing sleeve 24 by a bias application means 32. A sheet of transfer paper P is conveyed to reach a transfer station, where the back side (opposite side with respect to the photosensitive drum) of the transfer paper is charged by the transfer charger 23, whereby a developed image (toner image) 10 on the photosensitive drum surface is electrostatically transferred to the transfer paper P. The transfer paper P separated from the photosensitive drum 1 is sent to a hot pressure roller fixer 27 where the toner image on the transfer paper P is fixed.

Some magnetic developer remaining on the photosensitive drum 21 after the transfer step is removed by a cleaning device 28 equipped with a cleaning blade. The photosensitive drum 21 is discharged by an erasing exposure light source 26 and is subjected to a repeating cycle starting with the charging step by the primary charger 22.

The photosensitive drum 21 comprises an OPC photosensitive layer on an electroconductive substrate and rotates in the direction of the arrow. The developing sleeve 24 as a developer-carrying member comprising a non-magnetic cylinder rotates so as to move in the same direction as the photosensitive drum 21 surface at the developing station. Inside the developing sleeve 24 is disposed a multi-polar permanent magnet 240 (magnet roll) so as not to rotate. The multi-polar permanent magnet 240 may preferably be set to 500-900 Gauss at a pole N1, 600-1100 Gauss pole N2, 800-1500 Gauss at a pole S1 and 400-800 Gauss at a pole S2. The magnetic developer 30 in the developing device 29 is applied onto the developing sleeve 24 and the developer particles are provided with, e.g., a negative charge due to friction, e.g., between the developing sleeve 24 surface and the developer particles. The magnetic doctor blade 31 of iron is disposed in proximity with the cylindrical developing sleeve surface with a gap of about 50 microns to 500 microns and so as to confront one magnetic pole of the multi-polar permanent magnet, whereby a magnetic toner layer is formed in a thin and uniform thickness (30-300 microns) so that the magnetic developer layer is thinner than the gap between the photosensitive drum 21 and the developing sleeve 24 at the developing station. The revolution speed of the developing sleeve 24 is adjusted so that the sleeve surface velocity is substantially the same as or close to the speed of the photosensitive drum 21 surface. It is possible to compose the magnetic doctor blade 31 of a permanent magnet instead of iron. At the developing station, it is possible to apply an AC bias or a pulsed bias between the developing sleeve 24 and the photosensitive drum 21 surface by the biasing means 32. The AC bias may appropriately comprise a frequency f of 900-1600 Hz and a peak-to-peak voltage V<sub>pp</sub> of 1500-2300 V, and the DC bias may appropriately be -100 to -350 volts.

At the developing station, the developer particles are transferred to the photosensitive drum side while reciprocating between the developing sleeve 24 and the photosensitive drum 21 because of an electrostatic force exerted by the electrostatic image-bearing member surface and the action of the AC bias or pulsed bias electric field.

Instead of the magnetic doctor blade 31, an elastic blade formed of an elastic material such as silicone rub-

ber can also be used to apply the developer 300 n a regulated thickness onto the developing sleeve 24 under the action of a pressing force.

Instead of the OPC photosensitive drum, it is possible to use an insulating drum for electrostatic recording, or a photosensitive drum having a layer of a photoconductive insulating substance, such as a-Se, CdS, ZnO<sub>2</sub> or a-Si in appropriate selection depending on the developing conditions, as the photosensitive drum 21.

In the image forming apparatus, plural members inclusive of some of the above-mentioned members such as the photosensitive drum (image-bearing member), developing means, charging means and cleaning means can be integrally combined to form an apparatus unit so

15 that the unit can be connected to or released from the apparatus body. For example, at least one of the charging means, photosensitive drum and cleaning means can be integrally combined with the developing means to form a single unit so that it can be attached to or released from the apparatus body including the remainder of the image forming apparatus by a guide means such as a guide rail provided to the body. In this instance, it is also possible to compose such an apparatus unit by the charging means, cleaning means and/or photosensitive drum.

In case where the image forming apparatus according to the present invention is used as a printer for facsimile, the image light 25 as a latent image forming means may be replaced by digital light image of laser light for printing received data. FIG. 8 is a block diagram for illustrating such an embodiment.

Referring to FIG. 8, a controller 111 controls an image reader (or image reading unit) 110 and a printer 119. The entirety of the controller 111 is regulated by a CPU 117. Data read from the image reader 110 is transmitted through a transmitter circuit 113 to a remote terminal such as another facsimile machine. On the other hand, data received from a remote terminal is transmitted through a receiver circuit 112 to a printer 119. An image memory 116 stores prescribed image data. A printer controller 118 controls the printer 119. A telephone handset 114 is connected to the receiver circuit 112 and the transmitter circuit 113.

More specifically, an image received from a line (or circuit) 115 (i.e., image data received from a remote terminal connected by the line) is demodulated by means of the receiver circuit 112, decoded by the CPU 117, and sequentially stored in the image memory 116. When image data corresponding to at least one page is stored in the image memory 116, image recording or output is effected with respect to the corresponding page. The CPU 117 reads image data corresponding to one page from the image memory 116, and transmits the decoded data corresponding to one page to the printer controller 118. When the printer controller 118 receives the image data corresponding to one page from the CPU 117, the printer controller 118 controls the printer 119 so that image data recording corresponding to the page is effected. During the recording by the printer 119, the CPU 117 receives another image data corresponding to the next page.

As described above, the urea derivative according to the present invention is little liable to soil the developer-carrying member, is colorless or only light-colored, is thermally and mechanically stable and has good triboelectric chargeability.

Accordingly, the developer prepared by using the urea derivative is not readily affected by changes in

temperature and humidity and does not readily cause image quality deterioration during continuous copying, thus being able to provide images having an excellent uniformity of density. Further, the developer is excellent in storage stability and causes little decrease in triboelectric chargeability by a long term of storage. When the urea derivative is used to form a color toner, the color toner can provide clear images. Further, the urea derivative can have a remarkably different levels of triboelectric chargeability by using different kinds of 10 substituents so that the developer according to the present invention can be applied to a variety of developing methods.

### EXAMPLES

Hereinbelow, the present invention is described in more detail based on Examples. In the Examples, "part(s)" used in describing formulations are all by weight.

#### Example 1

|                                                       |               |
|-------------------------------------------------------|---------------|
| Styrene/n-butyl methacrylate copolymer                | 100 wt. parts |
| Carbon black                                          | 5 wt. parts   |
| Compound Example (1) in a parachloro-substituted form | 2 wt. parts   |

The above ingredients were well blended in a blender and kneaded through a twin-screw extruder set at 150° C. The kneaded product was cooled, coarsely crushed by a cutter mill and finely pulverized by a pulverizer using a jet air stream, followed by classification by means of a fixed wall-type wind force classifier. The resultant classified powder was further subjected to classification by a multi-division classifier ("Elbow Jet Classifier", available from Nittetsu Kogyo K.K.) for strict classification-removal of coarse powder fraction and ultra-fine powder fraction simultaneously, to recover black fine powder (toner) having a weight-average particle size of 8.5 microns. The thus obtained black fine powder contained 23% by number of particles having a particle size of 5 microns or below, 26% by number of particles having a particle size of 8-12.7 microns, and 0.3 wt. % of particles having a particle size of 16 microns or larger.

0.6 part of hydrophobic silica fine powder treated with dimethyldichlorosilane was added to 100 parts of the black fine powder, and the mixture was blended in a Henschel mixer to obtain a toner (containing silica fine powder). The toner in an amount of 5 g was mixed with 96 g of carrier to measure the triboelectric charge thereof by the flow-off method in a normal temperature/normal humidity environment of 23° C./60%RH, whereby a value of -28° C./g was obtained.

Then, 5 parts of the toner (with silica) was mixed with 100 parts of an acrylic resin-coated ferrite carrier having an average particle size of 65 microns to obtain a two-component type developer.

The two-component type developer was subjected to a copying test by using a commercially available color electrophotographic copier ("CLC-500", available from Canon K.K.).

As a result, under the normal temperature/normal humidity environmental conditions of 23° C./60%RH, clear black images having an image density of 1.51 were obtained from the initial stage and no deterioration was observed even after copying of 10<sup>4</sup> sheets.

Then, a similar copying test was performed under the low temperature/low humidity conditions of 15° C./10%RH, whereby images having a high density of 1.47 were obtained from the initial stage. Further, under the high temperature/high humidity conditions of 35° C./85%RH, good images having a density of 1.55 were obtained.

#### Example 2

Blue fine powder (toner) having a weight-average particle size of 8.3 microns was prepared and mixed with silica fine powder in the same manner as in Example 1 except that the 5 parts of carbon black was replaced by 4 parts of a copper phthalocyanine pigment (C.I. Pigment Blue 15). The toner (with silica) was further blended with the same carrier in the same ratio as in Example 1 to obtain a two-component type developer.

The developer was subjected to the same copying test as in Example 1 whereby, under the conditions of 23° C./60%RH, clear blue images free from fog and having a density of 1.56 were obtained from the initial stage. No image quality deterioration was observed even after copying of 10<sup>4</sup> sheets. As a result of the copying tests under 35° C./85%RH and 15° C./10%RH, similarly good results as under 23° C./60% RH were obtained.

#### Example 3

Red fine powder (toner) having a weight-average particle size of 8.2 microns was prepared and mixed with silica fine powder in the same manner as in Example 1 except that the 5 parts of carbon black was replaced by 4 parts of a quinacridone pigment (C.I. Pigment Red 122). The toner (with silica) was further blended with the same carrier in the same ratio as in Example 1 to obtain a two-component type developer.

The developer was subjected to the same copying test as in Example 1 whereby, under the conditions of 23° C./60%RH, clear magenta images free from fog and having a density of 1.57 were obtained from the initial stage. No image quality deterioration was observed even after copying of 10<sup>4</sup> sheets. As a result of the copying tests under 35° C./85%RH and 15° C./10%RH, similarly good results as under 23° C./60% were obtained.

#### Example 4

Yellow fine powder (toner) having a weight-average particle size of 8.1 microns was prepared and mixed with silica fine powder in the same manner as in Example 1 except that the 5 parts of carbon black was replaced by 4 parts of a yellow pigment (C.I. Pigment Yellow 17). The toner (with silica) in an amount of 6 parts was further blended with 100 parts of the same carrier as in Example 1 to obtain a two-component type developer.

The developer was subjected to the same copying test as in Example 1 whereby, under the conditions of 23° C./60%RH, clear yellow images free from fog and having a density of 1.53 were obtained from the initial stage. No image quality deterioration was observed even after copying of 10<sup>4</sup> sheets. As a result of the copying tests under 35° C./85%RH and 15° C./10%RH, similarly good results as under 23° C./60% were obtained.

Full color images were formed by using the black, cyan, magenta and yellow developers prepared by Ex-

amples 1-4, whereby clear full color images were provided with good color mixing characteristic and gradation characteristic.

#### Comparative Example 1

Black fine powder (toner) having a weight-average particle size of 8.4 microns was prepared and mixed with silica fine powder in the same manner as in Example 1 except that the 2 parts of Compound Example 1 was replaced by 2 parts of N,N'-bis(4-chlorophenyl)thiourea. The toner showed a triboelectric charge of -11  $\mu$ C/g as measured according to the same method as in Example 1. The toner (with silica) was further blended with the same carrier in the same ratio as in Example 1 to obtain a two-component type developer.

The developer was subjected to the same copying test as in Example 1 under the conditions of 23° C./60%RH, whereby an image having an image density of 1.39 was obtained. However, in the continuous copying test for examining durability, the image density was lowered to 1.20 on a 2000-th sheet which also showed ground fog in a practically problematic degree. As a result of inspection after the copying test, conspicuous toner scattering was observed in the copying apparatus, so that the toner was judged as commercially unacceptable.

#### Example 6

|                                                       |               |
|-------------------------------------------------------|---------------|
| Styrene/n-butyl methacrylate copolymer                | 100 wt. parts |
| Magnetic material                                     | 80 wt. parts  |
| Low-molecular weight polypropylene wax                | 3 wt. parts   |
| Compound Example (2) in a parafluoro-substituted form | 3 wt. parts   |

The above ingredients were well blended in a blender and kneaded through a twin-screw extruder set at 140° C. The kneaded product was cooled, coarsely crushed by a cutter mill and finely pulverized by a pulverizer using a jet air stream, followed by classification by means of a fixed wall-type wind force classifier. The resultant classified powder was further subjected to classification by a multi-division classifier ("Elbow Jet Classifier", available from Nittetsu Kogyo K.K.) for strict classification-removal of coarse powder fraction and ultra-fine powder fraction simultaneously, to recover black fine powder (toner) having a weight-average particle size of 8.3 microns.

0.6 part of hydrophobic silica fine powder treated with hexamethyldisilazane was added to 100 parts of the black fine powder, and the mixture was blended in a Henschel mixer to obtain a monocomponent-type developer.

The monocomponent-type developer thus obtained was subjected to a copying test by using a commercially available copying machine ("NP-6650", available from Canon K.K.) under the environmental conditions of 23° C./60% RH (normal temperature/normal humidity), whereby clear images free from fog and roughness having an image density of 1.41 were obtained at a resolution of 6.3 lines/mm. Further, on continuous copying of  $3 \times 10^4$  sheets for evaluation of durability, it was possible to obtain good images having an image density of 1.39 and a resolution of 6.3 lines/mm which were thus not inferior to the images at the initial stage. The triboelectric charge of the developer on the developing sleeve was measured to be -11.5  $\mu$ C/g at the initial stage and -10.7  $\mu$ C/g after copying  $3 \times 10^4$  sheets, and almost no soiling was observed on the sleeve.

Then, a copying test was performed under the conditions of 15° C./10%RH, similarly good images were obtained at a high density. Similarly good results were obtained in a continuous copying test of  $3 \times 10^4$  sheets. Similar copying test and continuous copying test were performed under the conditions of 35° C./85%RH, whereby good results were obtained. The developer was further left standing for 1 month under the conditions and then subjected to the same copying test and continuous copying test, whereby satisfactory results of no problem were obtained.

#### Example 7

Black fine powder (magnetic toner) having a weight-average particle size of 11.4 microns was prepared in the same manner as in Example 6 except that the 3 parts of Compound Example (2) was replaced by 3 parts of Compound Example (3) in a parachloro-substituted form and the amount of the magnetic material was reduced from 80 parts to 60 parts.

Then, 0.5 wt. part of hydrophobic silica fine powder treated with silicone oil was added to 100 parts of the black fine powder, followed by blending with a Henschel mixer, to obtain a monocomponent-type developer.

The monocomponent-type developer thus obtained was subjected to a copying test by using a commercially available copying machine ("NP-6650", available from Canon K.K.) under the environmental conditions of 23° C./60% RH (normal temperature/normal humidity), whereby clear images free from fog and roughness having a high image density of 1.40 were obtained. Further, on continuous copying of  $3 \times 10^4$  sheets for evaluation of durability, it was possible to obtain good images not inferior to the images at the initial stage. The triboelectric charge of the developer on the developing sleeve was measured to be -10.6  $\mu$ C/g at the initial stage and -10.2  $\mu$ C/g after copying  $3 \times 10^4$  sheets, and almost no soiling was observed on the sleeve. Then, a copying test was performed under the conditions of 15° C./10%RH, similarly good images were obtained at a high density. Similarly good results were obtained in a continuous copying test of  $3 \times 10^4$  sheets. Similar copying test and continuous copying test were performed under the conditions of 35° C./85%RH, whereby good results were obtained. The developer was further left standing for 1 month under the conditions and then subjected to the same copying test and continuous copying test, whereby satisfactory results of no problem were obtained.

#### Example 8

|                                                          |           |
|----------------------------------------------------------|-----------|
| Styrene/n-butyl methacrylate copolymer                   | 100 parts |
| Copper-phthalocyanine pigment (C. I. Pigment Blue 15)    | 5 parts   |
| Low-molecular weight polypropylene wax                   | 3 parts   |
| Compound Example (4) in an ortho-chloro-substituted form | 4 parts   |

A blue fine powder (toner) having a weight average particle size of 11.5 microns was prepared from the above ingredients otherwise in a similar manner as in Example 6.

0.5 wt. part of hydrophobic silica fine powder treated with dimethyldichlorosilane was added to 100 parts of the blue fine powder thus obtained, followed by blend-

ing by using a Henschel mixer to obtain a toner (with silica). Then, 7 parts of the toner (with silica) was blended with 100 parts of an acrylic resin-coated ferrite carrier having an average particle size of 65 microns to obtain a two-component type developer.

The two-component type developer thus obtained was subjected to a copying test using a commercially available copying machine ("NP-6650", available from Canon K.K.) under the environmental conditions of 23° C./60%RH, whereby good images having an image density of 1.35 were obtained. When the two-component type developer was evaluated with respect to durability by continuous copying of 5000 sheets, whereby good images not inferior to the images at the initial stage were obtained.

Then, copying tests were performed under the conditions of 15° C./10%RH, and the conditions of 35° C./85%RH, whereby similarly good results were obtained under the respective conditions.

#### Example 9

|                                                                  |           |
|------------------------------------------------------------------|-----------|
| Polyester (acid value: 9.5 mgKOH/g, hydroxyl value: 16.3 mgKOH/g | 100 parts |
| Carbon black                                                     | 5 parts   |
| Compound Example (5) in a meta-nitro-substituted form            | 2 parts   |

A black fine powder (toner) having a weight average particle size of 8.2 microns was prepared from the above ingredients otherwise in a similar manner as in Example 1.

0.6 wt. part of hydrophobic silica fine powder treated with hexamethyldisilazane was added to 100 parts of the black fine powder thus obtained, followed by blending by using a Henschel mixer to obtain a toner (with silica). Then, 6 parts of the toner (with silica) was blended with 100 parts of an acrylic resin-coated ferrite carrier having an average particle size of 65 microns to obtain a two-component type developer.

The two-component type developer thus obtained was subjected to a copying test using a commercially available color copying machine ("CLC-500", available from Canon K.K.) under the environmental conditions of 23° C./60%RH, whereby clear images having an image density of 1.42 were obtained from the initial stage, and no image quality deterioration was observed even after copying of 10<sup>4</sup> sheets.

As a result of a copying test under the conditions of 15° C./10%RH, images having a high density of 1.38 were obtained from the initial stage. Also under the conditions of 35° C./85%RH, good images having a density of 1.48 were obtained.

#### Example 10

|                                    |              |
|------------------------------------|--------------|
| Styrene/2-ethylhexyl acrylate      | 90 wt. parts |
| Styrene/butadiene copolymer        | 10 wt. parts |
| Magnetite                          | 75 wt. parts |
| Low-molecular weight polypropylene | 4 wt. parts  |

The above ingredients were well blended in a blender and kneaded through a twin-screw extruder set at 150° C. The kneaded product was cooled, coarsely crushed by a cutter mill and finely pulverized by a pulverizer using a jet air stream, followed by classification by means of a fixed wall-type wind force classifier. The resultant classified powder was further subjected to classification by a multi-division classifier ("Elbow Jet Classifier", available from Nittetsu Kogyo K.K.) for strict classification-removal of coarse powder fraction and ultra-fine powder fraction simultaneously, to recover black fine powder (toner) having a weight-average particle size of 8.1 microns.

"Classifier", available from Nittetsu Kogyo K.K.) for strict classification-removal of coarse powder fraction and ultra-fine powder fraction simultaneously, to recover fine powder having a weight-average particle size of 8.7 microns.

To 100 parts of the fine powder, 1.0 part of Compound Example (6) in a 4-fluoro-substituted form and 0.3 part of silica fine powder as additive materials were added, and the mixture was pre-treated by blending by a Henschel mixer.

Then, the mixture was subjected to 5 min. of an attaching-embedding treatment by means of an apparatus as shown in FIG. 5 under the conditions of a minimum blade clearance of 1 mm and a blade peripheral speed of 60 m/sec. As a result of observation of the treated product through an electron microscope, it was observed that the additive materials were attached to and partially embedded in the surface of the toner particles.

Further, to 100 parts of the thus treated product, 0.5 part of hydrophobic silica fine powder treated with hexamethyldisilazane was added and blended, to obtain a mono-component type developer.

The monocomponent-type developer thus obtained was subjected to a copying test by using a commercially available copying machine ("NP-6650", available from Canon K.K.) under the environmental conditions of 23° C./60% RH (normal temperature/normal humidity), whereby clear images free from fog and roughness having an image density of 1.38 were obtained at a resolution of 6.3 lines/mm. Further, on continuous copying of 2×10<sup>4</sup> sheets for evaluation of durability, it was possible to obtain good images having an image density of 1.32 which were thus not inferior to the images at the initial stage. Then, a copying test was performed under the conditions of 15° C./10%RH, similarly good images were obtained at a high density. Similarly good results were obtained in a continuous copying test of 2×10<sup>4</sup> sheets. Similar copying test and continuous copying test were performed under the conditions of 35° C./85%RH, whereby good results were obtained.

#### Example 11

|                                                       |               |
|-------------------------------------------------------|---------------|
| Styrene/n-butyl methacrylate copolymer                | 100 wt. parts |
| Magnetic material                                     | 80 wt. parts  |
| Low-molecular weight polypropylene wax                | 3 wt. parts   |
| Compound Example (2) in a parafluoro-substituted form | 1 wt. parts   |

The above ingredients were well blended in a blender and kneaded through a twin-screw extruder set at 140° C. The kneaded product was cooled, coarsely crushed by a cutter mill and finely pulverized by a pulverizer using a jet air stream, followed by classification by means of a fixed wall-type wind force classifier. The resultant classified powder was further subjected to classification by a multi-division classifier ("Elbow Jet Classifier", available from Nittetsu Kogyo K.K.) for strict classification-removal of coarse powder fraction and ultra-fine powder fraction simultaneously, to recover black fine powder (toner) having a weight-average particle size of 8.1 microns.

0.6 part of hydrophobic silica fine powder treated with dimethyl silicone oil was added to 100 parts of the black fine powder, and the mixture was blended in a

Henschel mixer to obtain a monocomponent-type developer.

The monocomponent-type developer thus obtained was subjected to a copying test by using a commercially available laser beam printer ("LBP-8II", available from Canon K.K.) under the environmental conditions of 23° C./60% RH (normal temperature/normal humidity), whereby clear images free from fog having an image density of 1.41 were obtained. Further, on continuous copying of 3000 sheets for evaluation of durability, it was possible to obtain good images having an image density of 1.40 which were thus not inferior to the images at the initial stage. Then, a copying test was performed under the conditions of 15° C./10%RH, similarly good images were obtained at a high density. Similarly good results were obtained in a continuous copying test of 3000 sheets. Similar copying test and continuous copying test were performed under the conditions of 35° C./85%RH, whereby good results were obtained.

#### Example 12

|                                                        |               |
|--------------------------------------------------------|---------------|
| Styrene/n-butyl methacrylate copolymer                 | 100 wt. parts |
| Carbon black                                           | 5 wt. parts   |
| Compound Example (21) in a paramethyl-substituted form | 2 wt. parts   |

The above ingredients were well blended in a blender and kneaded through a twin-screw extruder set at 150° C. The kneaded product was cooled, coarsely crushed by a cutter mill and finely pulverized by a pulverizer using a jet air stream, followed by classification by means of a fixed wall-type wind force classifier. The resultant classified powder was further subjected to classification by a multi-division classifier ("Elbow Jet Classifier", available from Nittetsu Kogyo K.K.) for strict classification-removal of coarse powder fraction and ultra-fine powder fraction simultaneously, to recover black fine powder (toner) having a weight-average particle size of 7.9 microns.

0.6 part of hydrophobic silica fine powder treated with dimethyldichlorosilane was added to 100 parts of the black fine powder, and the mixture was blended in a Henschel mixer to obtain a toner (containing silica fine powder). The triboelectric charge of the toner was measured to be -24 μC/g by the blow-off method.

Then, 5 parts of the toner (with silica) was mixed with 100 parts of an acrylic resin-coated ferrite carrier having an average particle size of 65 microns to obtain a two-component type developer.

The two-component type developer was subjected to a copying test by using a commercially available color electrophotographic copier ("CLC-500", available from Canon K.K.).

As a result, under the normal temperature/normal humidity environmental conditions of 23° C./60%RH, clear black images having an image density of 1.47 were obtained from the initial stage and no deterioration was observed even after copying of 10<sup>4</sup> sheets.

Then, a similar copying test was performed under the low temperature/low humidity conditions of 15° C./10%RH, whereby images having a high density of 1.43 were obtained from the initial stage. Further, under the high temperature/high humidity conditions of 35° C./85%RH, good images having a density of 1.52 were obtained.

#### Example 13

5 Blue fine powder (toner) having a weight-average particle size of 8.5 microns was prepared and mixed with silica fine powder in the same manner as in Example 12 except that the 5 parts of carbon black was replaced by 4 parts of a copper phthalocyanine pigment (C.I. Pigment Blue 15). The toner (with silica) was further blended with the same carrier in the same ratio as in Example 12 to obtain a two-component type developer.

10 The developer was subjected to the same copying test as in Example 12 whereby, under the conditions of 23° C./60%RH, clear blue images free from fog and having a density of 1.48 were obtained from the initial stage. No image quality deterioration was observed even after copying of 10<sup>4</sup> sheets. As a result of the copying tests under 35° C./85%RH and 15° C./10%RH, similarly good results as under 23° C./60% RH were obtained.

#### Example 14

15 Red fine powder (toner) having a weight-average particle size of 8.0 microns was prepared and mixed with silica fine powder in the same manner as in Example 12 except that the 5 parts of carbon black was replaced by 4 parts of a quinacridone pigment (C.I. Pigment Red 122). The toner (with silica) was further blended with the same carrier in the same ratio as in Example 12 to obtain a two-component type developer.

20 The developer was subjected to the same copying test as in Example 12 whereby, under the conditions of 23° C./60%RH, clear magenta images free from fog and having a density of 1.49 were obtained from the initial stage. No image quality deterioration was observed even after copying of 10<sup>4</sup> sheets. As a result of the copying tests under 35° C./85%RH and 15° C./10%RH, similarly good results as under 23° C./60% RH were obtained.

#### Example 15

25 Yellow fine powder (toner) having a weight-average particle size of 8.3 microns was prepared and mixed with silica fine powder in the same manner as in Example 12 except that the 5 parts of carbon black was replaced by 4 parts of a yellow pigment (C.I. Pigment Yellow 17). The toner (with silica) in an amount of 6 parts was further blended with 100 parts of the same carrier as in Example 12 to obtain a two-component type developer.

30 The developer was subjected to the same copying test as in Example 12 whereby, under the conditions of 23° C./60%RH, clear yellow images free from fog and having a density of 1.46 were obtained from the initial stage. No image quality deterioration was observed even after copying of 10<sup>4</sup> sheets. As a result of the copying tests under 35° C./85%RH and 15° C./10%RH, similarly good results as under 23° C./60% RH were obtained.

#### Example 16

35 Full color images were formed by using the black, cyan, magenta and yellow developers prepared by Examples 12-15, whereby clear full color images were provided with good color mixing characteristic and gradation characteristic.

## Example 17

|                                                            |               |
|------------------------------------------------------------|---------------|
| Styrene/n-butyl methacrylate copolymer                     | 100 wt. parts |
| Magnetic material                                          | 80 wt. parts  |
| Low-molecular weight polypropylene wax                     | 3 wt. parts   |
| Compound Example (22) in a paraiso-propyl-substituted form | 3 wt. parts   |

The above ingredients were well blended in a blender and kneaded through a twin-screw extruder set at 140° C. The kneaded product was cooled, coarsely crushed by a cutter mill and finely pulverized by a pulverizer using a jet air stream, followed by classification by means of a fixed wall-type wind force classifier. The resultant classified powder was further subjected to classification by a multi-division classifier ("Elbow Jet Classifier", available from Nittetsu Kogyo K.K.) for strict classification-removal of coarse powder fraction and ultra-fine powder fraction simultaneously, to recover black fine powder (toner) having a weight-average particle size of 8.0 microns.

0.6 part of hydrophobic silica fine powder treated with hexamethyldisilazane was added to 100 parts of the black fine powder, and the mixture was blended in a Henschel mixer to obtain a monocomponent-type developer.

The monocomponent-type developer thus obtained was subjected to a copying test by using a commercially available copying machine ("NP-6650", available from Canon K.K.) under the environmental conditions of 23° C./60% RH (normal temperature/normal humidity), whereby clear images free from fog and roughness having an image density of 1.39 were obtained at a resolution of 6.3 lines/mm. Further, on continuous copying of  $3 \times 10^4$  sheets for evaluation of durability, it was possible to obtain good images having an image density of 1.36 and a resolution of 6.3 lines/mm which were thus not inferior to the images at the initial stage. The triboelectric charge of the developer on the developing sleeve was measured to be  $-9.5 \mu\text{C/g}$  at the initial stage and  $-9.0 \mu\text{C/g}$  after copying  $3 \times 10^4$  sheets, and almost no soiling was observed on the sleeve. Then, a copying test was performed under the conditions of 15° C./10%RH, similarly good images were obtained at a high density. Similarly good results were obtained in a continuous copying test of  $3 \times 10^4$  sheets. Similar copying test and continuous copying test were performed under the conditions of 35° C./85%RH, whereby good results were obtained. The developer was further left standing for 1 month under the conditions and then subjected to the same copying test and continuous copying test, whereby satisfactory results of no problem were obtained.

## Example 18

Black fine powder (magnetic toner) having a weight-average particle size of 10.2 microns was prepared in the same manner as in Example 17 except that the 3 parts of Compound Example (22) was replaced by 3 parts of Compound Example (23) in a paramethoxy-substituted form and the amount of the magnetic material was reduced from 80 parts to 60 parts.

Then, 0.5 wt. part of hydrophobic silica fine powder treated with silicone oil was added to 100 parts of the black fine powder, followed by blending with a Henschel mixer, to obtain a monocomponent-type developer.

The monocomponent-type developer thus obtained was subjected to a copying test by using a commercially available copying machine ("NP-6650", available from Canon K.K.) under the environmental conditions of 23° C./60% RH (normal temperature/normal humidity), whereby clear images free from fog and roughness having a high image density of 1.36 were obtained. Further, on continuous copying of  $3 \times 10^4$  sheets for evaluation of durability, it was possible to obtain good images not inferior to the images at the initial stage. The triboelectric charge of the developer on the developing sleeve was measured to be  $-9.6 \mu\text{C/g}$  at the initial stage and  $-9.0 \mu\text{C/g}$  after copying  $3 \times 10^4$  sheets, and almost no soiling was observed on the sleeve. Then, a copying test was performed under the conditions of 15° C./10%RH, similarly good images were obtained at a high density. Similarly good results were obtained in a continuous copying test of  $3 \times 10^4$  sheets. Similar copying test and continuous copying test were performed under the conditions of 35° C./85%RH, whereby good results were obtained. The developer was further left standing for 1 month under the conditions and then subjected to the same copying test and continuous copying test, whereby satisfactory results of no problem were obtained.

## Example 19

|                                                          |           |
|----------------------------------------------------------|-----------|
| Styrene/n-butyl methacrylate copolymer                   | 100 parts |
| Copper-phthalocyanine pigment<br>(C. I. Pigment Blue 15) | 5 parts   |
| Low-molecular weight polypropylene wax                   | 3 parts   |
| Compound Example (24) in a ortho-ethyl-substituted form  | 4 parts   |

A blue fine powder (toner) having a weight average particle size of 11.7 microns was prepared from the above ingredients otherwise in a similar manner as in Example 17.

0.5 wt. part of hydrophobic silica fine powder treated with dimethylchlorosilane was added to 100 parts of the blue fine powder thus obtained, followed by blending by using a Henschel mixer to obtain a toner (with silica). Then, 7 parts of the toner (with silica) was blended with 100 parts of an acrylic resin-coated ferrite carrier having an average particle size of 65 microns to obtain a two-component type developer.

The two-component type developer thus obtained was subjected to a copying test using a commercially available copying machine ("NP-6650", available from Canon K.K.) under the environmental conditions of 23° C./60%RH, whereby good images having an image density of 1.32 were obtained. When the two-component type developer was evaluated with respect to durability by continuous copying of 5000 sheets, whereby good images not inferior to the images at the initial stage were obtained.

Then, copying tests were performed under the conditions of 15° C./10%, and the conditions of 35° C./85%RH, whereby similarly good results were obtained under the respective conditions.

## Example 20

|                                                                   |           |
|-------------------------------------------------------------------|-----------|
| Polyester (acid value: 9.5 mgKOH/g, hydroxyl value: 16.3 mgKOH/g) | 100 parts |
| Carbon black                                                      | 5 parts   |
| Compound Example (25) in a meta-                                  | 2 parts   |

A black fine powder (toner) having a weight average particle size of 7.7 microns was prepared from the above ingredients otherwise in a similar manner as in Example 12.

0.6 wt. part of hydrophobic silica fine powder treated with hexamethyldisilazane was added to 100 parts of the black fine powder thus obtained, followed by blending by using a Henschel mixer to obtain a toner (with silica). Then, 6 parts of the toner (with silica) was blended with 100 parts of an acrylic resin-coated ferrite carrier having an average particle size of 65 microns to obtain a two-component type developer.

The two-component type developer thus obtained was subjected to a copying test using a commercially available color copying machine ("CLC-500", available from Canon K.K.) under the environmental conditions of 23° C./60%RH, whereby clear images having an image density of 1.44 were obtained from the initial stage, and no image quality deterioration was observed even after copying of  $10^4$  sheets.

As a result of a copying test under the conditions of 15° C./10%RH, images having a high density of 1.36 were obtained from the initial stage. Also under the conditions of 35° C./85%RH, good images having a density of 1.48 were obtained.

#### Example 21

|                                    |              |
|------------------------------------|--------------|
| Styrene/2-ethylhexyl acrylate      | 90 wt. parts |
| Styrene/butadiene copolymer        | 10 wt. parts |
| Magnetite                          | 75 wt. parts |
| Low-molecular weight polypropylene | 4 wt. parts  |

The above ingredients were well blended in a blender and kneaded through a twin-screw extruder set at 150° C. The kneaded product was cooled, coarsely crushed by a cutter mill and finely pulverized by a pulverizer using a jet air stream, followed by classification by means of a fixed wall-type wind force classifier. The resultant classified powder was further subjected to classification by a multi-division classifier ("Elbow Jet Classifier", available from Nittetsu Kogyo K.K.) for strict classification-removal of coarse powder fraction and ultra-fine powder fraction simultaneously, to recover fine powder having a weight-average particle size of 8.7 microns.

To 100 parts of the fine powder, 1.0 part of Compound Example (26) in a 4-amino-substituted form and 0.3 part of silica fine powder as additive materials were added, and the mixture was pre-treated by blending by a Henschel mixer.

Then, the mixture was subjected to 5 min. of an attaching-embedding treatment by means of an apparatus as shown in FIG. 5 under the conditions of a minimum blade clearance of 1 mm and a blade peripheral speed of 60 m/sec. As a result of observation of the treated product through an electron microscope, it was observed that the additive materials including the 4-amino-substituted compound were attached to and partially embedded in the surface of the toner particles. Further, to 100 parts of the thus treated product, 0.5 part of hydrophobic silica fine powder treated with hexamethyldisilazane was added and blended, to obtain a mono-component type developer.

The monocomponent-type developer thus obtained was subjected to a copying test by using a commercially available copying machine ("NP-6650", available from Canon K.K.) under the environmental conditions of 23° C./60% RH (normal temperature/normal humidity), whereby clear images free from fog and roughness having an image density of 1.32 were obtained at a resolution of 6.3 lines/mm. Further, on continuous copying of  $2 \times 10^4$  sheets for evaluation of durability, it was possible to obtain good images having an image density of 1.28 which were thus not inferior to the images at the initial stage. Then, a copying test was performed under the conditions of 15° C./10%RH, similarly good images were obtained at a high density. Similarly good results were obtained in a continuous copying test of  $2 \times 10^4$  sheets. Similar copying test and continuous copying test were performed under the conditions of 35° C./85%RH, whereby good results were obtained.

#### Example 22

|                                                              |               |
|--------------------------------------------------------------|---------------|
| Styrene/n-butyl methacrylate copolymer                       | 100 wt. parts |
| Magnetic material                                            | 80 wt. parts  |
| Low-molecular weight polypropylene wax                       | 3 wt. parts   |
| Compound Example (22) in an ortho-isopropyl-substituted form | 1 wt. parts   |

The above ingredients were well blended in a blender and kneaded through a twin-screw extruder set at 140° C. The kneaded product was cooled, coarsely crushed by a cutter mill and finely pulverized by a pulverizer using a jet air stream, followed by classification by means of a fixed wall-type wind force classifier. The resultant classified powder was further subjected to classification by a multi-division classifier ("Elbow Jet Classifier", available from Nittetsu Kogyo K.K.) for strict classification-removal of coarse powder fraction and ultra-fine powder fraction simultaneously, to recover black fine powder (toner) having a weight-average particle size of 8.3 microns.

0.6 part of hydrophobic silica fine powder treated with dimethyl silicone oil was added to 100 parts of the black fine powder, and the mixture was blended in a Henschel mixer to obtain a monocomponent-type developer.

The monocomponent-type developer thus obtained was subjected to a copying test by using a commercially available laser beam printer ("LBP-8II", available from Canon K.K.) under the environmental conditions of 23° C./60% RH (normal temperature/normal humidity), whereby clear images free from fog having an image density of 1.37 were obtained. Further, on continuous copying of 3000 sheets for evaluation of durability, it was possible to obtain good images having an image density of 1.34 which were thus not inferior to the images at the initial stage. Then, a copying test was performed under the conditions of 15° C./10%RH, similarly good images were obtained at a high density. Similarly good results were obtained in a continuous copying test of 3000 sheets. Similar copying test and continuous copying test were performed under the conditions of 35° C./85%RH, whereby good results were obtained.

What is claimed is:

1. A developer for developing electrostatic images, comprising: a toner containing a binder resin and a charge controller, said charge controller comprising an

arylurea compound which comprises an arylurea having at least one electron-attracting group or electron-donating group, or a polyarylurea including such an arylurea as a recurring unit.

2. The developer according to claim 1, wherein said arylurea has an electron-attracting group.

3. The developer according to claim 2, wherein said arylurea comprises an N,N'-bisarylurea derivative represented by the following formula:



wherein Y<sup>1</sup> and Y<sup>2</sup> denote a phenyl or naphthyl group; R<sup>1</sup> and R<sup>2</sup> independently denote a halogen atom, nitro group, sulfonic acid group, carboxyl group, carboxylic acid ester group, cyano group or carbonyl group; R<sup>3</sup> and R<sup>4</sup> denote a hydrogen atom, alkyl group, alkoxy group, phenyl group capable of having a substituent, or aralkyl group capable of having a substituent; R<sup>5</sup> and R<sup>6</sup> denote a hydrogen atom or C<sub>1</sub>-C<sub>8</sub> hydrocarbon group; k and l are 0, 1 or 2 satisfying k+1  $\geq$  1; and m and n are 1 or 2.

4. The developer according to claim 2, which is a monocomponent-type developer comprising the toner.

5. The developer according to claim 4, wherein said arylurea comprises an N,N'-bisarylurea derivative represented by the following formula:



wherein Y<sup>1</sup> and Y<sup>2</sup> denote a phenyl or naphthyl group; R<sup>1</sup> and R<sup>2</sup> independently denote a halogen atom, nitro group, sulfonic acid group, carboxyl group, carboxylic acid ester group, cyano group or carbonyl group; R<sup>3</sup> and R<sup>4</sup> denote a hydrogen atom, alkyl group, alkoxy group, phenyl group capable of having a substituent, or 15 aralkyl group capable of having a substituent; R<sup>5</sup> and R<sup>6</sup> denote a hydrogen atom or C<sub>1</sub>-C<sub>8</sub> hydrocarbon group; k and l are 0, 1 or 2 satisfying k+1  $\geq$  l; and m and 20 n are 1 or 2.

25 6. The developer according to claim 4, wherein said  
arylurea compound comprises at least one compound  
selected from the group consisting of:



-continued



-continued



7. The developer according to claim 4, wherein said arylurea compound is internally added to the toner in a proportion of 0.1-10 wt. parts per 100 wt. parts of the binder resin.

8. The developer according to claim 4, wherein said arylurea compound is externally added to the toner in a proportion of 0.01-10 wt. parts per 100 wt. parts of the binder resin.

9. The developer according to claim 4, wherein said monocomponent-type developer comprises said toner and silica fine powder having BET specific surface area of at least 30 m<sup>2</sup>/g.

10. The developer according to claim 9, wherein said silica fine powder comprises hydrophobic silica fine powder having a hydrophobicity of 30-80.

11. The developer according to claim 4, wherein said toner contains a colorant.

12. The developer according to claim 4, wherein said toner is a color toner containing a colorant.

13. The developer according to claim 4, wherein said toner is a magnetic toner containing a magnetic material having an average particle size of 0.1-1 micron.

14. The developer according to claim 13, wherein said magnetic material is contained in the magnetic toner in a proportion of 40-150 wt. parts per 100 wt. parts of the binder resin.

15. The developer according to claim 4, wherein said binder resin comprises a styrene-acrylate copolymer.

16. The developer according to claim 4, wherein said binder resin comprises a styrene-methacrylate copolymer.

17. The developer according to claim 4, wherein said binder resin comprises a polyester resin.

18. The developer according to claim 4, wherein microns.

19. The developer according to claim 4, wherein said toner has a weight-average particle size of 4-10 microns and contains 12-60% by number of toner particles hav-

ing a particle size of 5 microns or smaller, 1-33% by number of toner particles having a particle size of 8-12.7 microns, and 2.0 wt. % or less of toner particles having a particle size of 16 microns or larger.

20. The developer according to claim 4, wherein said monocomponent-type developer contains at least one additive selected from the group consisting of lubricants, abrasives, fluidity-imparting agents, anti-caking agents, and electroconductivity-imparting agents.

21. The developer according to claim 4, wherein said toner contains a waxy substance.

22. The developer according to claim 2, which is a two-component-type developer comprising the toner and a carrier.

23. The developer according to claim 22, wherein said arylurea comprises an N,N'-bisarylurea derivative represented by the following formula:



20

wherein Y<sup>1</sup> and Y<sup>2</sup> denote a phenyl or naphthyl group; R<sup>1</sup> and R<sup>2</sup> independently denote a halogen atom, nitro group, sulfonic acid group, carboxyl group, carboxylic acid ester group, cyano group or carbonyl group; R<sup>3</sup> and R<sup>4</sup> denote a hydrogen atom, alkyl group, alkoxy group, phenyl group capable of having a substituent, or aralkyl group capable of having a substituent; R<sup>5</sup> and R<sup>6</sup> denote a hydrogen atom or C<sub>1</sub>-C<sub>8</sub> hydrocarbon group; k and l are 0, 1 or 2 satisfying k+1 ≥ 1; and m and n are 1 or 2.

24. The developer according to claim 22, wherein said arylurea compound comprises at least one compound selected from the group consisting of:



40



45



50



60



65

-continued



-continued



and



25. The developer according to claim 22, wherein said arylurea compound is internally added to the toner in a proportion of 0.1-10 wt. parts per 100 wt. parts of the binder resin.

26. The developer according to claim 22, wherein said arylurea compound is externally added to the toner in a proportion of 0.01-10 wt. parts per 100 wt. parts of the binder resin.

27. The developer according to claim 22, wherein said monocomponent-type developer comprises said toner and silica fine powder having BET specific surface area of at least 30 m<sup>2</sup>/g.

28. The developer according to claim 27, wherein said silica fine powder comprises hydrophobic silica fine powder having a hydrophobicity of 30-80.

29. The developer according to claim 22, wherein said toner contains a colorant.

30. The developer according to claim 22, wherein said toner is a color toner containing a colorant.

31. The developer according to claim 22, wherein said toner is a magnetic toner containing a magnetic material having an average particle size of 0.1-1 micron.

32. The developer according to claim 31, wherein said magnetic material is contained in the magnetic toner in a proportion of 40-150 wt. parts per 100 wt. parts of the binder resin.

33. The developer according to claim 22, wherein said binder resin comprises a styrene-acrylate copolymer.

34. The developer according to claim 22, wherein said binder resin comprises a styrene-methacrylate copolymer.

35. The developer according to claim 22, wherein said binder resin comprises a polyester resin.

36. The developer according to claim 22, wherein said toner has a weight-average particle size of 3-15 microns.

37. The developer according to claim 22, wherein said toner has a weight-average particle size of 4-10 microns and contains 12-60% by number of toner particles having a particle size of 5 microns or smaller,

1-33% by number of toner particles having a particle size of 8-12.7 microns, and 2.0 wt. % or less of toner particles having a particle size of 16 microns or larger.

5 38. The developer according to claim 22, wherein said monocomponent-type developer contains at least one additive selected from the group consisting of lubricants, abrasives, fluidity-imparting agents, anti-caking agents, and electroconductivity-imparting agents.

10 39. The developer according to claim 22, wherein said toner contains a waxy substance.

40. The developer according to claim 1, wherein said arylurea has an electron-donating group.

15 41. The developer according to claim 40, wherein said arylurea comprises an N,N'-bisarylurea derivative represented by the following formula:



20 25. wherein Y<sup>1</sup> and Y<sup>2</sup> denote a phenyl group, naphthyl group or anthryl group; R<sup>1</sup> and R<sup>2</sup> independently denote an alkyl group, alkoxy group or amino group; R<sup>3</sup> and R<sup>4</sup> denote a hydrogen atom, alkyl group, alkoxy group, amino group, phenyl group capable of having a substituent, or aralkyl group capable of having a substituent; R<sup>5</sup> and R<sup>6</sup> are a hydrogen atom or C<sub>1</sub>-C<sub>8</sub> hydrocarbon group; k and l are 0, 1 or 2 satisfying k+1 $\geq$ 1; and m and n are 1 or 2.

30 35. 42. The developer according to claim 40, which is a monocomponent-type developer comprising the toner.

40 43. The developer according to claim 42, wherein said arylurea comprises an N,N'-bisarylurea derivative represented by the following formula:



50 55. wherein Y<sup>1</sup> and Y<sup>2</sup> denote a phenyl group, naphthyl group or anthryl group; R<sup>1</sup> and R<sup>2</sup> independently denote an alkyl group, alkoxy group or amino group; R<sup>3</sup> and R<sup>4</sup> denote a hydrogen atom, alkyl group, alkoxy group, amino group, phenyl group capable of having a substituent, or aralkyl group capable of having a substituent; R<sup>5</sup> and R<sup>6</sup> are a hydrogen atom or C<sub>1</sub>-C<sub>8</sub> hydrocarbon group; k and l are 0, 1 or 2 satisfying k+1 $\geq$ 1; and m and n are 1 or 2.

35 44. The developer according to claim 42, wherein said arylurea compound comprises at least one compound selected from the group consisting of:





and



5 45. The developer according to claim 42, wherein  
10 said arylurea compound is internally added to the toner  
in a proportion of 0.1-10 wt. parts per 100 wt. parts of  
the binder resin.

15 46. The developer according to claim 42, wherein  
said arylurea compound is externally added to the toner  
in a proportion of 0.01-10 wt. parts per 100 wt. parts of  
the binder resin.

20 47. The developer according to claim 42, wherein  
said monocomponent-type developer comprises said  
toner and silica fine powder having BET specific sur-  
face area of at least 30 m<sup>2</sup>/g.

25 48. The developer according to claim 47, wherein  
said silica fine powder comprises hydrophobic silica  
fine powder having a hydrophobicity of 30-80.

49. The developer according to claim 42, wherein  
said toner contains a colorant.

50. The developer according to claim 42, wherein  
said toner is a color toner containing a colorant.

30 51. The developer according to claim 42, wherein  
said toner is a magnetic toner containing a magnetic  
micron.

35 52. The developer according to claim 51, wherein  
said magnetic material is contained in the magnetic  
toner in a proportion of 40-150 wt. parts per 100 wt.  
parts of the binder resin.

53. The developer according to claim 42, wherein  
said binder resin comprises a styrene-acrylate copoly-  
mer.

40 54. The developer according to claim 42, wherein  
said binder resin comprises a styrene-methacrylate co-  
polymer.

55. The developer according to claim 42, wherein  
said binder resin comprises a polyester resin.

45 56. The developer according to claim 42, wherein  
said toner has a weight-average particle size of 3-15  
microns.

57. The developer according to claim 42, wherein  
50 said toner has a weight-average particle size of 4-10  
microns and contains 12-60% by number of toner parti-  
cles having a particle size of 5 microns or smaller,  
1-33% by number of toner particles having a particle  
size of 8-12.7 microns, and 2.0 wt. % or less of toner  
55 particles having a particle size of 16 microns or larger.

58. The developer according to claim 42, wherein  
said monocomponent-type developer contains at least  
one additive selected from the group consisting of lubri-  
cants, abrasives, fluidity-imparting agents, anti-caking  
60 agents, and electroconductivity-imparting agents.

59. The developer according to claim 42, wherein  
said toner contains a waxy substance.

60. The developer according to claim 40, which is a  
monocomponent-type developer comprising the toner.

65 61. The developer according to claim 60, wherein  
said arylurea comprises an N,N'-bisarylurea derivative  
represented by the following formula:



5

wherein  $Y^1$  and  $Y^2$  denote a phenyl group, naphthyl group or anthryl group;  $R^1$  and  $R^2$  independently denote an alkyl group, alkoxy group or amino group;  $R^3$  and  $R^4$  denote a hydrogen atom, alkyl group, alkoxy group, amino group, phenyl group capable of having a substituent, or aralkyl group capable of having a substituent;  $R^5$  and  $R^6$  are a hydrogen atom or  $C_1-C_8$  hydrocarbon group;  $k$  and  $l$  are 0, 1 or 2 satisfying  $k+l \leq 1$ ; and  $m$  and  $n$  are 1 or 2.

62. The developer according to claim 60, wherein said arylurea compound comprises at least one compound selected from the group consisting of:



-continued



and



30 63. The developer according to claim 60, wherein said arylurea compound is internally added to the toner in a proportion of 0.1-10 wt. parts per 100 wt. parts of the binder resin.

35 64. The developer according to claim 60, wherein said arylurea compound is externally added to the toner in a proportion of 0.01-10 wt. parts per 100 wt. parts of the binder resin.

40 65. The developer according to claim 60, wherein said monocomponent-type developer comprises said toner and silica fine powder having BET specific surface area of at least  $30 \text{ m}^2/\text{g}$ .

45 66. The developer according to claim 65, wherein said silica fine powder comprises hydrophobic silica fine powder having a hydrophobicity of 30-80.

67. The developer according to claim 60, wherein said toner contains a colorant.

68. The developer according to claim 60, wherein said toner is a color toner containing a colorant.

50 69. The developer according to claim 60, wherein said toner is a magnetic toner containing a magnetic material having an average particle size of 0.1-1 micron.

70. The developer according to claim 69, wherein said magnetic material is contained in the magnetic toner in a proportion of 40-150 wt. parts per 100 wt. parts of the binder resin.

55 71. The developer according to claim 60, wherein said binder resin comprises a styrene-acrylate copolymer.

60 72. The developer according to claim 60, wherein said binder resin comprises a styrene-methacrylate copolymer.

73. The developer according to claim 60, wherein said binder resin comprises a polyester resin.

65 74. The developer according to claim 60, wherein said toner has a weight-average particle size of 3-15 microns.

75. The developer according to claim 60, wherein said toner has a weight-average particle size of 4-10 microns and contains 12-60% by number of toner particles having a particle size of 5 microns or smaller, 1-33% by number of toner particles having a particle size of 8-12.7 microns, and 2.0 wt. % or less of toner particles having a particle size of 16 microns or larger.

76. The developer according to claim 60, wherein

said monocomponent-type developer contains at least one additive selected from the group consisting of lubricants, abrasives, fluidity-imparting agents, anti-caking agents, and electroconductivity-imparting agents.

77. The developer according to claim 70, wherein said toner contains a waxy substance.

\* \* \* \* \*

10

15

20

25

30

35

40

45

50

55

60

65

UNITED STATES PATENT AND TRADEMARK OFFICE  
CERTIFICATE OF CORRECTION

PATENT NO. : 5,288,579

DATED : February 22, 1994

INVENTOR(S) : KATSUHIKO TANAKA, ET AL.

Page 1 of 4

It is certified that error appears in the above-identified patent and that said Letters Patent is hereby corrected as shown below:

COLUMN 1

Line 61, "changes" should read --changes---.

COLUMN 2

Line 59, "image-bearing" should read --image-bearing member--.

COLUMN 3

Line 26, "According" should read --According to--.

Line 39, "compound" should read --Compound--.

COLUMN 4

Line 67, "enumerated hereinbelow," should read  
--enumerated,--

COLUMN 7

Line 52, "electron-dona" should read --electron-donating--.

Line 53, "tive" should be deleted.

Line 54, "enumerated hereinbelow, should read  
--enumerated,--.

COLUMN 9

Line 45, "42 hours" should read --24 hours--.

UNITED STATES PATENT AND TRADEMARK OFFICE  
CERTIFICATE OF CORRECTION

PATENT NO. : 5,288,579

DATED : February 22, 1994

INVENTOR(S) : KATSUHIKO TANAKA, ET AL.

Page 2 of 4

It is certified that error appears in the above-identified patent and that said Letters Patent is hereby corrected as shown below:

COLUMN 10

Line 1, "form a" should read --form of--.  
Line 2, "synthesized identified" should read  
--synthesized and identified--.  
Line 58, "flame" should read --flame---.

COLUMN 11

Line 36, "thylchlorsilane," should read  
--thylchlorosilane,--.

COLUMN 12

Line 35, "derivative" should read --derivatives--.

COLUMN 13

Line 10, "aluminum" should read --aluminum,--.  
Line 11, "zinc," should be deleted.  
Line 13, "mixture" should read --mixtures--.  
Line 27, "2.0 wt." should read --2.0 wt. %--.  
Line 29, "particle" should read --the particle--.  
Line 41, "ISOTONR-II" should read --ISOTON<sup>R</sup>-II--.

COLUMN 15

Line 33, "Gauss pole" should read --Gauss at a pole--.

COLUMN 16

Line 1, "n" should read --in--.

UNITED STATES PATENT AND TRADEMARK OFFICE  
CERTIFICATE OF CORRECTION

PATENT NO. : 5,288,579

DATED : February 22, 1994

INVENTOR(S) : KATSUHIKO TANAKA, ET AL.

Page 3 of 4

It is certified that error appears in the above-identified patent and that said Letters Patent is hereby corrected as shown below:

COLUMN 17

Line 9, "a" should be deleted.

Line 54, "-28°C./g" should read -- -28  $\mu$ C./g--.

Line 68, "10<sup>4</sup> sheets" should read --10<sup>4</sup> sheets--.

COLUMN 20

Line 44, "3 $\times$ 10<sup>4</sup> sheets" should read --3 $\times$ 10<sup>4</sup> sheets--.

Line 58, "a" should read --an--.

COLUMN 22

Line 22, "mono-component" should read --monocomponent--.

Line 49, "1 wt. parts" should read --1 wt. part--.

COLUMN 24

Line 18, "15°C./10RH," should read --15°C./10% RH,--.

COLUMN 26

Line 33, "a" should read --an--.

Line 53, "obtained" should read --obtained--.

COLUMN 27

Line 67, "mono-compo-" should read --monocompo- --.

COLUMN 28

Line 16, "2 $\times$ 10<sup>4</sup> sheets" should read --2 $\times$ 10<sup>4</sup> sheets--.

Line 26, "1 wt. parts" should read --1 wt. part--.

UNITED STATES PATENT AND TRADEMARK OFFICE  
CERTIFICATE OF CORRECTION

PATENT NO. : 5,288,579

DATED : February 22, 1994

INVENTOR(S) : KATSUHIKO TANAKA, ET AL.

Page 4 of 4

It is certified that error appears in the above-identified patent and that said Letters Patent is hereby corrected as shown below:

COLUMN 34

Line 64, "wherein" should read --wherein said toner has a weight-average particle size of 3-15--.

COLUMN 40

Line 30, "magnetic" (second occurrence) should read --magnetic material having an average particle size of 0.1-1--.

Signed and Sealed this

Thirteenth Day of September, 1994

Attest:



BRUCE LEHMAN

Attesting Officer

Commissioner of Patents and Trademarks